

## UNITED STATES PATENT OFFICE

2,543,006

## SMOKE AGENT

Leo Finkelstein, Aberdeen, and Sidney J. Magram, Baltimore, Md., assignors to the United States of America as represented by the Secretary of War

No Drawing. Application November 8, 1943,  
Serial No. 509,506

3 Claims. (Cl. 52—23)

(Granted under the act of March 3, 1883, as amended April 30, 1928; 370 O. G. 757)

1

The invention described herein may be manufactured and used by or for the Government for governmental purposes, without the payment to us of any royalty thereon.

This invention relates to a colored smoke-forming composition.

The object of this invention is to provide an economical smoke-producing mixture which is particularly efficient when used in a smoke grenade or candle but which may also be effectively utilized in artillery or mortar projectiles, and in smoke pots or various other pyrotechnical devices.

The smoke-forming composition of this invention comprises as principal ingredients a mixture of a suitable dye, a fuel containing potassium chlorate and sulfur, and a combustion-controlling agent, such as sodium bicarbonate or potassium bicarbonate.

In the late war, small, portable, nonmissile devices which produced smoke by progressive burning of a chemical filling were known as smoke candles. Devices of larger size, not so readily portable but producing a more enduring smoke cloud with longer burning by virtue of their size, were called smoke pots. More recently, the smoke candles were developed along the lines of tear gas grenades and became known as smoke grenades. The grenades are a very convenient type of munition. They are easily carried by troops, and they are readily set into action after projection by small arms or when thrown by hand. However, the use of grenades for colored smoke had the serious limitation that known smoke mixtures were unsuitable in being too slow in igniting, too fast in burning, and erratic in burning.

The colored smoke-forming composition of the present invention does not have the limitations of previously known mixtures and has proved to be an efficient filling for utilization in the same kind of container as is used for tear gas grenades.

The composition has been satisfactorily standardized into one type with the following variety of colors:

- |           |           |
|-----------|-----------|
| 1. Yellow | 4. Green  |
| 2. Orange | 5. Blue   |
| 3. Red    | 6. Violet |

In producing the smoke-forming compositions, it is preferable to have a dry, uniform mixture of the ingredients and to use the ingredients in certain optimum proportions for forming a large amount of smoke.

Examples of satisfactory compositions are as follows:

2

Example 1.—Yellow smoke mixture

|                      | Percent |
|----------------------|---------|
| Auramine             | 38      |
| KClO <sub>3</sub> —S | 33.5    |
| NaHCO <sub>3</sub>   | 28.5    |

Example 2.—Orange smoke mixture

|                      | Percent |
|----------------------|---------|
| Orange dye           | 45      |
| KClO <sub>3</sub> —S | 31      |
| NaHCO <sub>3</sub>   | 24      |

The orange dye consists of a mixture of 39 parts of 8-chloro-1-aminoanthraquinone and 6 parts of auramine.

Example 3.—Red smoke mixture

|                            | Percent |
|----------------------------|---------|
| 1-methylaminoanthraquinone | 40      |
| KClO <sub>3</sub> —S       | 41      |
| NaHCO <sub>3</sub>         | 19      |

Example 4.—Green smoke mixture

|                      | Percent |
|----------------------|---------|
| Green dye            | 41      |
| KClO <sub>3</sub> —S | 36      |
| NaHCO <sub>3</sub>   | 23      |

The green dye consists of 29 parts of 1, 4-di-p-toluidino anthraquinone and 12 parts of auramine.

Example 5.—Blue smoke mixture

|                      | Percent |
|----------------------|---------|
| Indigo               | 64      |
| KClO <sub>3</sub> —S | 28      |
| NaHCO <sub>3</sub>   | 8       |

Example 6.—Violet smoke mixture

|                      | Percent |
|----------------------|---------|
| Violet dye           | 44      |
| KClO <sub>3</sub> —S | 42      |
| NaHCO <sub>3</sub>   | 14      |

The violet dye consists of a mixture of 26 parts of 1,4-diamino-2,3-dihydro anthraquinone and 18 parts of crude 1-methylaminoanthraquinone.

The fuel mixture preferably contains about 72% potassium chlorate and about 28% sulfur.

The following particle sizes are used in the formulations of the foregoing examples, but the particle sizes may be varied depending on the change in composition and on the burning time desired:

Potassium chlorate:

|                                                   |
|---------------------------------------------------|
| 85% minimum passes a No. 100 U. S. Standard sieve |
| 40% minimum passes a No. 200 U. S. Standard sieve |

**Sulfur:**

99% minimum passes a No. 100 U. S. Standard sieve  
 85% minimum passes a No. 200 U. S. Standard sieve

**Sodium bicarbonate:**

99% minimum passes a No. 100 U. S. Standard sieve  
 50% minimum passes a No. 200 U. S. Standard sieve

**Yellow dye:**

70% minimum passes a No. 100 U. S. Standard sieve  
 20% maximum passes a No. 200 U. S. Standard sieve

**Orange dye:**

92% minimum passes a No. 100 U. S. Standard sieve  
 16% minimum passes a No. 200 U. S. Standard sieve

**Red dye:**

90% minimum passes a No. 100 U. S. Standard sieve  
 70% minimum passes a No. 200 U. S. Standard sieve

**Green dye:**

95% minimum passes a No. 100 U. S. Standard sieve  
 40% minimum passes a No. 200 U. S. Standard sieve

**Blue dye:**

90% minimum passes a No. 100 U. S. Standard sieve  
 30% minimum passes a No. 200 U. S. Standard sieve

**Violet dye:**

95% minimum passes a No. 100 U. S. Standard sieve  
 60% minimum passes a No. 200 U. S. Standard sieve

Each of the smoke mixture charges may be loaded into a grenade body and compressed therein under a high pressure, e. g., pressure of 475 pounds per square inch. On top the smoke charge in the grenade body may be placed a starter charge formulated from silicon potassium nitrate and charcoal with a binder solution of cellulose nitrate and acetone. The starter mixture may be contained in a starter cup and be ignited by an ordinary grenade fuse made up of a primer and a train of black powder, the primer being set off by mechanical impact of a striker. The smoke mixture may be in any suitable container without a starter cup and can be ignited directly simply by a fuse.

In the operation of a colored smoke grenade, heat evolved by the chemical reaction of the fuel ingredients volatilizes the dye; and the dye vapors dispersed into the atmosphere condense to form a thick colored smoke. The colored smoke, if formed in sufficient volume and lasting for sufficient time, can be observed from long distances and serves as a signal, identification or for a variety of other purposes.

It is found to be extremely important to have the combustion reaction in the smoke mixture controlled in order to keep the temperature sufficiently low to prevent excessive decomposition and flaming of the dye. In general, the dye is an organic substance capable of being ignited at an elevated temperature. The dyes selected should be volatile and thermally stable at the temperature of the burning mixture.

The kinds of dyes found most suitable are commercial dyes as well as dyes specially made; it was found that some anthraquinone dyes, a diphenyl methane dye, an indigo dye and other vat-type dyes could be used.

The use of the agent for controlling the combustion reaction is very important. By moderating the temperature of the reaction without adversely affecting the ignition properties of the mixture, the agent makes possible the selection of suitable organic dyes, lengthens the time of burning and increases the smoke-developing efficiency of the mixture. A characteristic of the combustion-controlling agent is the property of decomposing when heated to within the temperature range of about 100° C. to 350° C., more preferably in the range of 200° C. to 300° C. Compounds having this characteristic are basic alkali bicarbonates, such as sodium bicarbonate and potassium bicarbonate.

It is to be understood that the invention is not limited by the specific examples and that various modifications are included within the scope of the invention.

**25 We claim:**

1. A colored smoke forming composition comprising a dry fuel mixture of sulfur and potassium chloride, a combustion controlling agent in a proportion of from about 8% to 28.5% NaHCO<sub>3</sub> and a dyestuff consisting by weight of from not less than 35% nor more than 45% of said composition selected from a group consisting of 1 methylaminoanthraquinone, 1,4-diamino-2,3-dihydro anthraquinone and a mixture of each of 35 said quinones.

2. A colored smoke forming composition comprising a dry fuel mixture of sulfur and potassium chloride, a combustion controlling agent in a proportion of from about 8% to 28.5% NaHCO<sub>3</sub> and a dyestuff consisting by weight of from not less than 35% nor more than 45% of said composition consisting of 1 methylaminoanthraquinone.

3. A colored smoke forming composition comprising of a dry fuel mixture of sulfur and potassium chloride, a combustion controlling agent in a proportion of from about 8% to 28.5% NaHCO<sub>3</sub> and a dyestuff consisting by weight of from not less than 35% nor more than 45% of said composition selected from 1,4-diamino-2,3-dihydro anthraquinone.

LEO FINKELSTEIN.  
 SIDNEY J. MAGRAM.

**REFERENCES CITED**

The following references are of record in the file of this patent:

**UNITED STATES PATENTS**

60 Number Name Date  
 1,319,329 Gowdy \_\_\_\_\_ Oct. 21, 1919  
 1,448,073 Lucas et al. \_\_\_\_\_ Mar. 13, 1923

**FOREIGN PATENTS**

65 Number Country Date  
 128,986 Great Britain \_\_\_\_\_ July 10, 1919

**OTHER REFERENCES**

Chemical Formulary—Bennett. Chem. Pub. Co. N. Y., vol. 4, 1939, page 444 (Copy in Scientific Library).

La Nature for 1940, pages 240-244 ("Les Nuages et Fumees Dans La Guerre Moderne").